



US005750296A

# United States Patent [19]

Kim et al.

[11] Patent Number: 5,750,296

[45] Date of Patent: May 12, 1998

[54] PHOTO-CONDUCTIVE COMPOSITION AND  
CRT BULB HAVING PHOTO-CONDUCTIVE  
LAYER FORMED OF THE SAME

3-35246 2/1991 Japan 430/83  
2095416 9/1982 United Kingdom

[75] Inventors: **Min-ho Kim**, Suwon; **Bong-mo Jeong**,  
**Jae-ho Shim**, both of Seoul; **Wan-woo**,  
**Park**, Yongin; **Deuk-yong Yang**,  
Suwon, all of Rep. of Korea

Primary Examiner—**Roland Martin**  
Attorney, Agent, or Firm—**Leydig, Voit & Mayer, Ltd.**

[73] Assignee: **Samsung Display Devices Co., Ltd.**,  
Kyungki-do, Rep. of Korea

[57] ABSTRACT

[21] Appl. No.: 696,786

[22] Filed: Aug. 14, 1996

[30] Foreign Application Priority Data

Dec. 29, 1995 [KR] Rep. of Korea 95-66819

[51] Int. Cl.<sup>6</sup> G03C 5/00; G03G 5/09

[52] U.S. Cl. 430/28; 430/83

[58] Field of Search 430/28, 83

[56] References Cited

U.S. PATENT DOCUMENTS

- |           |         |                 |         |
|-----------|---------|-----------------|---------|
| 4,362,798 | 12/1982 | Anderson et al. | 430/59  |
| 4,423,129 | 12/1983 | Takasu et al.   | 430/59  |
| 4,465,857 | 8/1984  | Neumann et al.  | 564/251 |
| 4,535,043 | 8/1985  | Ishikawa et al. | 430/58  |
| 4,784,929 | 11/1988 | Ueda et al.     | 430/83  |
| 4,865,934 | 9/1989  | Ueda et al.     | 430/59  |

FOREIGN PATENT DOCUMENTS

- |           |        |       |        |
|-----------|--------|-------|--------|
| 59-142556 | 8/1984 | Japan | 430/83 |
|-----------|--------|-------|--------|



where  $\text{R}_1$  is selected from the group consisting of a phenyl group substituted by one to three substituents selected from the group consisting of amino, dialkylamino,  $\text{C}_1-\text{C}_6$  alkoxy,  $\text{C}_1-\text{C}_6$  alkyl and cyano groups; 9-alkyl carbazole group; naphthyl group, and  $\text{R}_2$  and  $\text{R}_3$  are same or different independently from each other, each being selected from the group consisting of hydrogen and  $\text{C}_1-\text{C}_6$  alkyl, phenyl and naphthyl groups, and  $n$  is between 0 and 2; 1–15 wt % of a charge generating substance which absorbs light in the wavelength range of an ultraviolet region; 70–94 wt % of a binder; and 0.05–1 wt % of a surfactant. The photoconductive composition exhibits excellent sintering characteristic and can form a photoconductive layer having excellent coating properties, durability and luminance.

5 Claims, No Drawings

PHOTO-CONDUCTIVE COMPOSITION AND  
CRT BULB HAVING PHOTO-CONDUCTIVE  
LAYER FORMED OF THE SAME

BACKGROUND OF THE INVENTION

1. Field of the Invention

The present invention relates to a photo-conductive composition and a cathode ray tube (CRT) bulb having a photo-conductive layer formed of the same, and more particularly, to a photo-conductive composition for forming a photoconductive layer having excellent coating properties, durability and luminance, and a CRT bulb having a photo-conductive layer formed of the same.

2. Description of Related Art

A photo-conductive composition has been used in various fields applying electrophotographic technique such as photocopies and laser printers, and especially for the phosphor screen of a color cathode ray tube. Here, the phosphor screen of a cathode ray tube can be manufactured by a slurry coating method or an electrophotographic process.

In the slurry coating method, a panel is cleaned and then slurries of primary color (i.e., green, blue and red) emitting phosphors are respectively coated on the panel. Each phosphor slurry contains polyvinylalcohol (as its main component), ammonium dichromate and one of green-, blue-, and red-emitting phosphors. A predetermined portion of the coated panel is exposed through a shadow mask and developed, to give a phosphor screen in a dotted or striped pattern.

The above method, however, has certain problems. First, the phosphor remains at an unexposed portion in a relatively large amount after the developing step, so that the remaining phosphor is mixed with the phosphor to be coated later. Second, a reaction between the polyvinylalcohol and ammonium dichromate contained in the phosphor slurry produces a coloring substance, which deteriorates color purity.

As another method for manufacturing the phosphor screen for a cathode ray tube, a method using an electrophotographic technique is known. This method is not only simpler than the slurry method, but can also provide a color cathode ray tube having better luminance. In this method, a conductive layer is first formed on the inner surface of a panel using a spin coating method, and a photo-conductive layer is formed thereon. The photo-conductive layer is electrified with a corona charger, and a predetermined portion thereof is then exposed through a shadow mask. The exposed portion of the photo-conductive layer was controlled to be an electrically neutral condition, and green-, blue- and red phosphor compositions were respectively adhered to the unexposed portion thereof, to form a phosphor screen.

A photo-conductor includes a charge generating substance (CGM) and a charge transmitting substance (CTM). Thus, the photo-conductor behaves as an insulator in the dark, but exhibits electrical characteristics upon receiving light (UV or visible light), by releasing an electron or generating a hole.

An inorganic photo-conductor performs poorly in terms of sensitivity, thermal stability, durability and hygroresistance—besides being toxic. Further, the inorganic photo-conductor generates a great amount of residue during a sintering process, resulting in a photo-conductive layer having poor luminance. Therefore, the inorganic photo-conductor is not used substantially. Accordingly, an organic photo-conductor has recently been developed. An organic photo-conductor is lightweight, transparent and easy

to fire. However, the organic photo-conductor also exhibits a low electrification potential and poor charge generation and charge transmission ability.

In general, a photo-conductor composition comprises a charge generating substance, a charge transmitting substance and a binder. So far, Polyvinylcarbazole is frequently used as the charge generating substance. However, polyvinylcarbazole has the following disadvantages. That is, its charge potential is low and the luminance of the resulting cathode ray tube is reduced since some residue remains after a sintering process. Also, polyvinylcarbazole absorbs light in the wavelength range of the visible region, so that a manipulation with polyvinylcarbazole should be achieved in a darkroom, which obstructs its applicability. In addition, solvents such as chlorobenzene and cyclopentanone used for dissolving polyvinylcarbazole are not preferable, in view of the environment, worker's health and solvent cost.

Other charge transmitting substances are disclosed in U.S. Pat. No. 5,370,952, but are difficult to prepare and are environmentally hazardous.

SUMMARY OF THE INVENTION

An object of the present invention is to provide a photo-conductive composition for forming a photoconductive layer having excellent coating properties and durability, and luminance.

Another object of the present invention is to provide a cathode ray tube bulb having an enhanced luminance by adopting a photo-conductor layer formed from a photo-conductive composition having an excellent sintering characteristic.

To achieve the object, there is provided a photo-conductive composition comprising:

5-15 wt % of a charge transmitting substance, represented by the structural formula (1);



where  $\text{R}_1$  is selected from the group consisting of a phenyl group substituted by one to three substituents selected from the group consisting of amino, dialkylamino,  $\text{C}_1-\text{C}_6$  alkoxy,  $\text{C}_1-\text{C}_6$  alkyl and cyano groups; 9-alkyl carbazole group; naphthyl group, and  $\text{R}_2$  and  $\text{R}_3$  are the same or differ independently from each other, each being selected from the group consisting of hydrogen and  $\text{C}_1-\text{C}_6$  alkyl, phenyl and naphthyl groups, and  $n$  is between 0 and 2;

1-15 wt % of a charge generating substance which absorbs light in the wavelength range of an ultraviolet region;

70-94 wt % of a binder; and

0.05-1 wt % of a surfactant.

The other object of the present invention is achieved by a CRT bulb comprising a face plate on which a conductive layer, a photo-conductive layer and a phosphor screen are sequentially formed, a funnel which is connected to the face plate and provided with an electron gun and a deflection yoke, wherein the photo-conductive layer is formed of a composition comprising:

5-15 wt % of a charge transmitting substance, represented by the structural formula (1);



where  $R_1$  is selected from the group consisting of a phenyl group substituted by one to three substituents selected from the group consisting of amino, dialkylamino,  $C_1-C_6$  alkoxy,  $C_1-C_6$  alkyl and cyano groups; 9-alkyl carbazole group; naphthyl group, and  $R_2$  and  $R_3$  are same or different independently from each other, each being selected from the group consisting of hydrogen atom and  $C_1-C_6$  alkyl, phenyl and naphthyl groups, and  $n$  is between 0 and 2;

15 1-15 wt % of a charge generating substance which absorbs light in the wavelength range of an ultraviolet region;

70-94 wt % of a binder; and  
0.05-1 wt % of a surfactant.

#### DETAILED DESCRIPTION OF THE INVENTION

A photo-conductive composition of the present invention is characterized by a hydrazone compound of the structural formula (1) as a charge transmitting substance.

A typical hydrazone compound of the structural formula (1) includes 4-(diethylamino)benzaldehyde N-methyl-N-phenylhydrazone (2), 4-ethoxybenzaldehyde N,N-diphenylhydrazone (3), 4-(diethylamino)benzaldehyde N,N-diphenylhydrazone (4), 4-(diethylamino)benzaldehyde N,N-dimethylhydrazone (5), 9-ethyl-3-carbazolecarboxaldehyde N,N-diphenylhydrazone (6), and 2-methyl-4-(diethylamino)phenylaldehyde N,N-diphenylhydrazone (7).



-continued



The above hydrazone compounds are easily prepared and are considerably soluble in a usual organic solvents. Also, the residual potential is low and photo-conductive characteristics do not nearly change, even though photo-conductive layer formed of these hydrazone compounds is repetitively used. Further, since their absorption wavelength range corresponds to the ultraviolet region, yellow light (560-580 nm) is available for working.

Substances used as a charge generating substance absorb light in the wavelength range of an ultraviolet region and includes 3,5-dinitrobenzonitrile (8), 2,6-dichloroquinone-N-chloroimide (9), 2,6-dibromoquinone-N-chloroimide (10), mordant orange 1 (11), 3,3',4,4'-benzophenone tetracarboxylic dianhydride (12), and crystal violet lactone (13).





As the binder, polymethylmethacrylate, polycarbonate, polybutylmethacrylate or polystyrene is used.

Preferably, in coating a photo-conductive composition on the inner surface of a panel, a surfactant is added to the composition in a small amount, to reduce surface tension of the composition. Silicon silar 100 (available from General Electronics Co.) or Pluronic P-84 (available from BASF, Co.) is mainly used as the surfactant.

The solvent used for a photo-conductive composition includes chloroform, methylenechloride, acetone, toluene, cyclohexanone and cyclopentanone.

Hereinbelow, as an example for using the photo-conductive composition of the present invention, a method for manufacturing a phosphor screen of a color cathode ray tube by an electrophotographic technique will be described.

First, an inner surface of a panel of a cathode ray tube is cleaned and a conductive composition is coated thereon, to form a conductive layer. As a conductors for forming the conductive layer, an inorganic conductor such as tin oxide, indium oxide and indium tin oxide, or an organic conductor such as quaternary ammonium salts is used. Considering a thermal decomposition property during a sintering process, the organic conductor is preferably used.

The photo-conductive composition, comprising 5-15 wt % of a charge transmitting substance represented by the structural formula (1), 1-15 wt % of a charge generating substance which absorbs light in the wavelength range of an ultraviolet region, 70-94 wt % of a binder and 0.05-1 wt % of a surfactant, is coated on the conductive layer, to form a photo-conductive layer having a thickness of 2-6  $\mu\text{m}$ . Preferably, to prevent swelling of an aluminum layer after a sintering process, the photo-conductive layer should be formed in a thickness not exceeding 6  $\mu\text{m}$ .

The photo-conductive layer is electrified with a corona charger and a predetermined portion thereof is exposed through a shadow mask. The exposed portion of the photo-conductive layer is controlled to be an electrically neutral condition, and green-, blue- and red emitting phosphor compositions are adhered to the unexposed portion thereof, respectively. The phosphors are semi-solidified by using a highly-volatile solvent such as acetone and alcohol. The phosphors are completely fused on the resulting panel of the cathode ray tube by using an infrared heater, to thereby form a phosphor screen.

Hereinbelow, the present invention is described more concretely with respect to its examples intended to illustrate the instant invention without limiting the scope thereof.

#### (EXAMPLE 1)

After an inner surface of a panel was cleaned, a conductive layer was formed thereon. A photo-conductive composition, comprising 15 g of 4-(diethylamino)benzaldehyde N,N-dimethylphenylhydrazone, 10 g of 3,5-dinitrobenzonitrile, 100 g of polymethylmethacrylate, 1 g of

silicon silar 100 and 900 g of cyclohexanone, was coated on the conductive layer, to form a photo-conductive layer having a thickness of about 4  $\mu\text{m}$ . The photo-conductive layer was electrified with a corona charger, to obtain a surface potential between 200V and 600V.

A predetermined portion of the photo-conductive layer was exposed through a photo mask. The exposed portion of the photo-conductive layer was controlled to be an electrically neutral condition, and green-, blue- and red light emitting phosphor compositions were adhered to the unexposed portion thereof, respectively. The phosphors were semi-solidified by using acetone as a solvent and completely fused on the resulting panel of the cathode ray tube by heating at 70  $^{\circ}\text{C}$ . for twenty seconds, with an infrared heater, to form a phosphor screen.

#### (EXAMPLE 2)

A phosphor screen was formed according to the same method as described in Example 1 except that a photo-conductive composition comprising 15 g of 4-(diethylamino)benzaldehyde N,N-dimethylphenylhydrazone, 10 g of mordant orange 1, 100 g of polymethylmethacrylate, 1 g of silicon silar 100 and 900 g of cyclohexanone was used.

#### (EXAMPLE 3)

A phosphor screen was formed according to the same method as described in Example 1 except that a photo-conductive composition comprising 10 g of 2-methyl-4-(diethylamino)phenylaldehyde N,N-diphenylhydrazone, 10 g of 3,5-dinitrobenzonitrile, 100 g of polymethylmethacrylate, 1 g of silicon silar 100 and 900 g of cyclohexanone was used.

#### (Comparative Example)

After an inner surface of a panel was cleaned, a conductive layer was then formed thereon. Thereafter, a photo-conductive composition comprising 200 g of polyvinylcarbazole, 10 g of polymethylmethacrylate, 1 g of Celestin Blue and 3800 g of chlorobenzene was coated on the conductive layer, to thus form a layer having a thickness of about 4  $\mu\text{m}$ .

The predetermined portion of the photo-conductive layer was exposed through a shadow mask. The exposed portion of the photo-conductive layer was controlled to be an electrically neutral condition, and green-, blue- and red light emitting phosphor compositions were respectively adhered to the unexposed portion thereof, to form a phosphor screen.

Photo-conductive compositions of examples and comparative example were coated on the inner surface of a panel, respectively and then sintered, and the result was investigated in each case. In the comparative example, a great amount of residue was left after the sintering process, however, in the examples, the amount of residue was decreased. And, the residual potential of the examples was 10V or lower even after electrification and exposure are repetitively performed.

The present invention has the following advantages.

First, the photo-conductive composition according to the present invention has excellent durability and coating properties and prevents deterioration of luminance of a cathode ray tube by reducing the amount of residue left after a sintering process in a process for manufacturing CRT.

Second, a hydrazone compound as a charge transmitting substance is easy and cheap to prepare and yellow light is available for working, resulting in high mass production productivity.

What is claimed is:

1. A photo-conductive composition comprising:  
5–15 wt % of a charge transmitting substance, represented  
by the structural formula (1);



where  $R_1$  is selected from the group consisting of a phenyl group substituted by one to three substituents selected from the group consisting of amino, dialkylamino,  $C_1-C_6$  alkoxy,  $C_1-C_6$  alkyl and cyano groups; 9-alkyl carbazole group; naphthyl group, and  $R_2$  and  $R_3$  are same or different independently from each other, each being selected from the group consisting of hydrogen and  $C_1-C_6$  alkyl, phenyl and naphthyl groups, and  $n$  is between 0 and 2;

15 1–15 wt % of a charge generating substance having an ultraviolet absorption wavelength;

70–94 wt % of a binder; and

0.05–1 wt % of a surfactant.

2. A photo-conductive composition as claimed in claim 1, wherein said charge transmitting substance is one selected from the group consisting of 4-(diethylamino)benzaldehyde N-methyl-N-phenylhydrazone, 4-ethoxybenzaldehyde N,N-diphenylhydrazone, 4-(diethylamino)benzaldehyde N,N-diphenylhydrazone, 4-(diethylamino)benzaldehyde N,N-dimethylhydrazone, 9-ethyl-3-carbazolecarboxaldehyde N,N-diphenylhydrazone, and 2-methyl-4-(diethylamino)phenylaldehyde N,N-diphenylhydrazone.

3. A photo-conductive composition as claimed in claim 1, wherein said charge generating substance is one selected from the group consisting of 3,5-dinitrobenzonitrile, 2,6-dichloroquinone-N-chloroimide, 2,6-dibromoquinone-N-chloroimide, mordant orange 1, 3,3',4,4'-benzophenone tetracarboxylic dianhydride, and crystal violet lactone.

4. A photo-conductive composition as claimed in claim 1, wherein said binder is one selected from the group consisting of polymethacrylate, polycarbonate, polybutylmethacrylate and polystyrene.

5 5. A CRT bulb comprising a face plate on which a conductive layer, a photo-conductive layer and a phosphor screen are sequentially formed, a funnel which is connected to said face plate and provided with an electron gun and a deflection yoke, wherein said photo-conductive layer is formed of a composition comprising:

- 10 5–15 wt % of a charge transmitting substance, represented by the structural formula (1);



20 20 where  $R_1$  is selected from the group consisting of a phenyl group substituted by one to three substituents selected from the group consisting of amino, dialkylamino,  $C_1-C_6$  alkoxy,  $C_1-C_6$  alkyl and cyano groups; 9-alkyl carbazole group; naphthyl group, and  $R_2$  and  $R_3$  are same or different independently from each other, each being selected from the group consisting of hydrogen and  $C_1-C_6$  alkyl, phenyl and naphthyl groups, and  $n$  is between 0 and 2;

25 1–15 wt % of a charge generating substance which absorbs light in the wavelength range of an ultraviolet region;

30 70–94 wt % of a binder; and

0.05–1 wt % of a surfactant.

\* \* \* \* \*